



US011608541B2

(12) **United States Patent**  
**Zhang et al.**

(10) **Patent No.:** **US 11,608,541 B2**  
(45) **Date of Patent:** **Mar. 21, 2023**

(54) **MANUFACTURING METHOD FOR HIGH SILICON GRAIN ORIENTED ELECTRICAL STEEL SHEET**

(71) Applicant: **BAOSHAN IRON & STEEL CO., LTD.**, Shanghai (CN)

(72) Inventors: **Huabing Zhang**, Shanghai (CN); **Shuangjie Chu**, Shanghai (CN); **Guobao Li**, Shanghai (CN); **Wen Xiao**, Shanghai (CN); **Baojun Liu**, Shanghai (CN); **Yongjie Yang**, Shanghai (CN); **Kanyi Shen**, Shanghai (CN); **Dan Han**, Shanghai (CN); **Zhining Hu**, Shanghai (CN)

(73) Assignee: **BAOSHAN IRON & STEEL CO., LTD.**, Shanghai (CN)

(\*) Notice: Subject to any disclaimer, the term of this patent is extended or adjusted under 35 U.S.C. 154(b) by 150 days.

(21) Appl. No.: **17/040,684**

(22) PCT Filed: **Mar. 25, 2019**

(86) PCT No.: **PCT/CN2019/079442**

§ 371 (c)(1),  
(2) Date: **Sep. 23, 2020**

(87) PCT Pub. No.: **WO2019/184838**

PCT Pub. Date: **Oct. 3, 2019**

(65) **Prior Publication Data**

US 2021/0047706 A1 Feb. 18, 2021

(30) **Foreign Application Priority Data**

Mar. 29, 2018 (CN) ..... 201810272499.X

(51) **Int. Cl.**

**C21D 9/46** (2006.01)  
**C21D 6/00** (2006.01)

(Continued)

(52) **U.S. Cl.**  
CPC ..... **C21D 9/46** (2013.01); **C21D 6/008** (2013.01); **C21D 8/1222** (2013.01);  
(Continued)

(58) **Field of Classification Search**  
CPC ..... C21D 9/46; C21D 6/008; C21D 8/1222;  
C21D 8/1233; C21D 8/1255;  
(Continued)

(56) **References Cited**

U.S. PATENT DOCUMENTS

2014/0342094 A1 \* 11/2014 Hofener ..... C23C 24/04  
427/446

FOREIGN PATENT DOCUMENTS

CN 1692164 11/2005  
CN 1692164 A \* 11/2005 ..... C21D 8/1277  
(Continued)

OTHER PUBLICATIONS

International Search Report and Written Opinion dated Jun. 6, 2019 for PCT Patent Application No. PCT/CN2019/079442.

Primary Examiner — Anthony M Liang

Assistant Examiner — Danny N Kang

(74) Attorney, Agent, or Firm — Lei Fang, Esq.; Smith Tempel Blaha LLC

(57) **ABSTRACT**

Disclosed is a manufacturing method for a high silicon grain oriented electrical steel sheet, the silicon content of the high silicon grain oriented electrical steel is greater than 4 wt %, comprising the steps of: (1) performing decarburization annealing of a cold-rolled steel plate; (2) allowing high silicon alloy particles in a completely solid state to collide at a high speed with the surface of the decarburization annealed steel plate to be sprayed, thus forming a high silicon alloy coating on the surface of the steel plate to be sprayed; (3) coating a release agent and drying; and (4) annealing. The manufacturing method for the high silicon

(Continued)



grain oriented electrical steel sheet of the present invention is inexpensive, and, the high silicon grain oriented electrical steel sheet produced is of stable quality and is provided with great magnetic performance.

**14 Claims, 1 Drawing Sheet****(51) Int. Cl.**

*C22C 38/00* (2006.01)  
*C21D 8/12* (2006.01)  
*C22C 38/02* (2006.01)  
*C22C 38/04* (2006.01)  
*C22C 38/06* (2006.01)

**(52) U.S. Cl.**

CPC ..... *C21D 8/1233* (2013.01); *C21D 8/1255* (2013.01); *C21D 8/1272* (2013.01); *C21D 8/1283* (2013.01); *C22C 38/001* (2013.01); *C22C 38/02* (2013.01); *C22C 38/04*

(2013.01); *C22C 38/04* (2013.01); *C22C 38/06* (2013.01); *C21D 2201/05* (2013.01); *C22C 2202/02* (2013.01)

**(58) Field of Classification Search**

CPC ..... C21D 8/1272; C21D 8/1283; C21D 2201/05; C21D 1/76; C21D 8/1205; C21D 8/1261; C21D 8/1277; C21D 8/1288; C21D 8/12; C22C 38/001; C22C 38/002; C22C 38/02; C22C 38/04; C22C 38/06; C22C 2202/02; C23C 10/46; C23C 10/30; C23C 24/04

See application file for complete search history.

**(56)****References Cited**

## FOREIGN PATENT DOCUMENTS

|    |             |                 |
|----|-------------|-----------------|
| CN | 1692165     | 11/2005         |
| CN | 107338432   | 11/2017         |
| CN | 107338432 A | * 11/2017 ..... |
| JP | H0643607    | 6/1994          |

\* cited by examiner



**MANUFACTURING METHOD FOR HIGH SILICON GRAIN ORIENTED ELECTRICAL STEEL SHEET**

**CROSS-REFERENCE TO RELATED APPLICATIONS**

This application is a 371 U.S. National Phase of PCT International Application No. PCT/CN2019/079442 filed on Mar. 25, 2019, which claims benefit and priority to Chinese patent application no. 201810272499.X filed on Mar. 29, 2018, which is incorporated by reference herein in its entirety.

**TECHNICAL FIELD**

The invention relates to a method for manufacturing an electrical steel plate, and particularly to a method for manufacturing a grain-oriented electrical steel plate.

**BACKGROUND OF INVENTION**

Electrical steel plates are generally divided into grain-oriented electrical steel plates and non-oriented electrical steel plates. Among them, the grain-oriented electrical steel plate has a silicon content of about 3 wt % and a crystal texture with a grain orientation of (110)[001]. It has excellent magnetic performance along the rolling direction and can be used as core materials of transformers, engines, generators and other electronic equipment.

In recent years, operating frequency of some electronic and electrical components are increased for improving the efficiency, sensitivity and size reduction, and thus the demand for iron core materials having excellent high-frequency magnetic properties are gradually increased. The high silicon steel plate containing 6.5 wt % of Si has a magnetostriction coefficient ( $\lambda_s$ ) of approximate zero, thus has a significantly reduced iron loss under high frequency, a high maximum magnetic permeability ( $\mu_m$ ), and a low magnetic induction coercive force ( $H_c$ ), which is most suitable for manufacturing motors and audios with high-speed and high-frequency, high-frequency transformers, choke coils, and magnetic shields at high frequencies, and can also be used for reducing engine energy consumption and improve engine efficiency.

However, high silicon steel plate cannot be produced by conventional processes as hot rolling, cold rolling and annealing of the prior art. In the prior art, Chinese patent publication CN107217129A, dated Sep. 29, 2017, titled as "High silicon steel plate with excellent processability and magnetic properties and production method thereof", discloses a method for manufacturing a high silicon steel plate, wherein vertical double-rollers are used to directly cast high silicon strips having a thickness of 5 mm or less and Si content of 4%-7%, Al content of 0.5%-3%, and mixture of Si and Al content of 4.5%-8%, followed by hot rolling, cold rolling and annealing processes to obtain the final product. Chinese patent publication CN1692164A dated Nov. 2, 2005, titled as "A method for manufacturing a high silicon grain-oriented electrical steel plate with an excellent iron loss performance", discloses a high silicon grain-oriented electrical steel plate, wherein, based on conventional method for manufacturing oriented-silicon steel, the surface of the decarburization annealed steel plate is coated with a slurry silicified powder coating agent, and then the silicon diffusion reaction is activated during the high-temperature annealing at 1200° C. to obtain the high silicon steel plate. Although

the products manufactured by the methods above have excellent magnetic properties, a mass production by the method is difficult due to facts such as high manufacturing costs and unstable product quality, thus the method is difficult for commercialization.

Based on this, it is expected to obtain a method for manufacturing a high silicon grain-oriented electrical steel plate that is of low cost, and the manufactured high silicon grain-oriented electrical steel plate has stable quality and excellent magnetic properties.

**SUMMARY OF INVENTION**

15 The purpose of the invention is to provide a method for manufacturing a high silicon grain-oriented electrical steel plate that is of low cost, and the manufactured high silicon grain-oriented electrical steel plate has stable quality and excellent magnetic properties.

20 To achieve the above purpose, the invention provides a method for manufacturing a high silicon grain-oriented electrical steel plate, wherein the high silicon grain-oriented electrical steel plate has a silicon content of greater than 4 wt %, the method comprising steps of:

25 (1) performing a decarburization annealing with cold-rolled steel plate;  
 (2) having high silicon alloy particles of complete solid state collide with the surface of the decarburization annealed steel plate to be sprayed at high speed, so as to form a high silicon alloy coating on the surface of the steel plate to be sprayed;

30 (3) coating a separation agent and drying;  
 (4) annealing.

In step (2) of the above method, that is, during the cold spray process, the high silicon alloy particles do not melt before colliding with the surface of the steel plate to be sprayed at high speed. The high silicon alloy particles undergo strong plastic deformation in the micro-region of the surface of the steel plate to be sprayed during the collision, and their kinetic energy is converted into thermal energy and strain energy, thus depositing on the surface of the steel plate to be sprayed to form a high-silicon alloy coating. In step (3), in some embodiments, the separation agent may be mainly composed of  $MgO$ ,  $Al_2O_3$  or a mixture of both. Since in the method of the present invention, it is not necessary to form magnesium silicate base layer ( $Mg_2SiO_4$ ) as in the conventional process for manufacturing the grain-oriented electrical steel plate, the separation agent with lower activity than conventional such as  $MgO$  can be used.

35 40 45 50 Further, the method for manufacturing a high silicon grain-oriented electrical steel plate according to the present invention, wherein in step (2), the high silicon alloy particles have a Si content of 10-50 wt %.

In the method of the present invention, the inventor of the invention finds through research that when the high silicon alloy particles have a Si content less than 10 wt %, in order to produce the high silicon grain-oriented electrical steel plate of the present invention, it is necessary to increase the thickness of the high silicon alloy coating and prolong the subsequent silicon diffusion period during high-temperature annealing, resulting in a decrease in production efficiency. When the high silicon alloy particles have a Si content more than 50 wt %, the plastic deformation ability of the high silicon alloy particles is weakened, making it more difficult for forming the silicon alloy coating. Therefore, the inventor of the invention limits the element Si content in the high silicon alloy particles to 10-50 wt %.

Further, the method for manufacturing a high silicon grain-oriented electrical steel plate according to the present invention, wherein in step (2), the high silicon alloy particles have a particle size of 1-80  $\mu\text{m}$ .

In the method of the present invention, the inventor of the invention finds through research that if the high silicon alloy particles have a particle size less than 1  $\mu\text{m}$ , the manufacturing cost of the high silicon alloy particles will increase, and the surface of the high silicon alloy particles will be easily oxidized. When the high silicon alloy particles have a particle size greater than 80  $\mu\text{m}$ , it is difficult for the high silicon alloy particles to be accelerated to the critical speed for bonding during the spraying process. Therefore, the inventor of the invention limits the particle size of the high silicon alloy particles to 1-80  $\mu\text{m}$ .

Further, the method for manufacturing a high silicon grain-oriented electrical steel plate according to the present invention, wherein in step (2), the high silicon alloy particles of complete solid state collide with the surface of the decarburization annealed steel plate to be sprayed at a speed of 500-900 m/s.

In the method of the present invention, the inventor of the invention finds through research that when the collision speed of high silicon alloy particles is lower than 500 m/s, only erosion occurs without bonding, and when the collision speed of high silicon alloy particles is higher than 900 m/s, the high silicon alloy particles will corrode the high silicon grain-oriented electrical steel plate. Therefore, the inventor of the invention controls the collision speed of the high-silicon alloy particles at 500-900 m/s.

Further, the method for manufacturing a high silicon grain-oriented electrical steel plate according to the present invention, wherein in step (2), the high silicon alloy particles are driven by jet flow of working gas to collide with the surface of the decarburization annealed steel plate to be sprayed.

Further, the method for manufacturing a high silicon grain-oriented electrical steel plate according to the present invention, wherein in step (2), the working gas is nitrogen, helium or mixture of nitrogen and helium.

Further, the method for manufacturing a high silicon grain-oriented electrical steel plate according to the present invention, wherein in step (2), the high silicon alloy particles and working gas are ejected via a nozzle onto the surface of the steel plate to be sprayed so that the high silicon alloy particles of complete solid state collide with the surface of the decarburization annealed steel plate to be sprayed at high speed.

Further, the method for manufacturing a high silicon grain-oriented electrical steel plate according to the present invention, wherein in step (2), the temperature of the high silicon alloy particles at the outlet of the nozzle is controlled as 80-500° C.

In the method of the present invention, the inventor of the invention finds through research that when the temperature of the high silicon alloy particles at the outlet of the nozzle is lower than 80° C., the effect of increasing the adhesion cannot be achieved due to low temperature, and when the temperature of the high silicon alloy particles is higher than 500° C., the high silicon alloy particles are easily oxidized, which in turn leads to an increase in surface defects of the final high silicon steel plate. Therefore, the inventor of the invention limits the temperature of the high silicon alloy particles at the outlet of the nozzle within the range of 80-500° C.

Further, the method for manufacturing a high silicon grain-oriented electrical steel plate according to the present

invention, wherein in step (2), the working gas is heated to 200-700° C. and then is sent to the nozzle.

In the above technical solution, heating the gas can increase the speed of the high silicon alloy particles, and also make the high silicon alloy particles have a certain temperature, so that the high silicon alloy particles are more prone to plastic deformation when they collide with the steel plate to be sprayed.

Further, the method for manufacturing a high silicon grain-oriented electrical steel plate according to the present invention, wherein in step (2), the nozzle is Laval nozzle.

Further, the method for manufacturing a high silicon grain-oriented electrical steel plate according to the present invention, wherein in step (2), the outlet of the nozzle is set 10-60 mm away from the surface of the steel plate to be sprayed.

In the method of the present invention, in order to prevent the deceleration and excessive oxidation of the high silicon alloy particles in the working gas, the distance between the outlet of the nozzle and the surface of the steel plate to be sprayed is limited to 10-60 mm.

Further, the method for manufacturing a high silicon grain-oriented electrical steel plate according to the present invention, wherein in step (2), the high silicon alloy coating is formed on surface of one side or both sides of the steel plate to be sprayed, and the thickness of the high silicon alloy coating satisfies the following formula:

$$T_c/T_s \geq (x1-x2)/(x3-x1)$$

wherein  $T_c$  is the thickness of the high silicon alloy coating, in  $\mu\text{m}$ , and when the high silicon alloy coating is formed on both sides of the steel plate, the thickness of the high silicon alloy coating is the sum of coating thickness of two sides of the steel plate;  $T_s$  is the thickness of the decarburization annealed steel plate to be sprayed, in  $\mu\text{m}$ ;  $x1$  is target silicon content of the high silicon grain-oriented electrical steel plate, in wt %;  $x2$  is an initial silicon content of the steel plate to be sprayed, in wt %;  $x3$  is the silicon content of the high silicon alloy particles, in wt %.

When the thickness of coating satisfies  $T_c/T_s < (x1-x2)/(x3-x1)$ , the total silicon content contained in the steel plate and alloy coating will be lower than the target silicon content of the high silicon grain-oriented electrical steel plate, which is impossible to obtain the desired high silicon steel plate through subsequent siliconizing treatment, and considering such factors as the inevitable voids in the coating and the stability of subsequent siliconizing, it is required that  $T_c/T_s \geq (x1-x2)/(x3-x1)$ . Under conditions where other process parameters are stable, the thickness of coating  $T_c$  is usually controlled accurately to make the actual silicon content in the steel plate approach to the target silicon content. Further, in the method for manufacturing a high silicon grain-oriented electrical steel plate according to the present invention, in the step (1), the total oxygen content on the surface of the decarburization annealed steel plate to be sprayed is controlled as less than 700 ppm, the element C content being controlled as less than 50 ppm, and the dew point of the decarburization annealing step is controlled as 40-65° C.

In the method of the present invention, the total oxygen content on the surface of the decarburization annealed steel plate to be sprayed is controlled as less than 700 ppm, and the element C content is less than 50 ppm. The inventor of the invention finds through research that when the dew point of the decarburization annealing step is controlled as 40-65° C., the decarburization effect can be ensured so as to eliminate the magnetic aging of the final product, and the formation of oxide film on the surface of the steel plate can

be inhibited. On one hand, it is beneficial for the high silicon alloy particles to be combined with the decarburization annealed steel plate. On the other hand, it is also beneficial for the high silicon alloy coating to infiltrate toward the decarburization annealed steel plate to be sprayed with silicon during the annealing process of step (4). Since the high silicon alloy coating is formed, the surface of the steel plate has sufficient roughness, so that the coating ability of the insulating coating in the insulating coating process that may be contained after step (4) can be guaranteed, without forming magnesium silicate base layer as in the conventional process for manufacturing the grain-oriented electrical steel plate. Therefore the total oxygen content on the surface of the steel plate to be sprayed is less than that of the conventional process.

Further, the method for manufacturing a high silicon grain-oriented electrical steel plate according to the present invention, wherein in step (4), implementing a secondary recrystallization at an annealing temperature above 1100° C. and in a N<sub>2</sub>+H<sub>2</sub> atmosphere, and then evenly heating the steel plate at temperature above 1150° C. for at least 20 hours and in a reducing atmosphere having a H<sub>2</sub> content over 90%, so as to achieve a uniform diffusion of element Si.

Further, the method for manufacturing a high silicon grain-oriented electrical steel plate according to the present invention, wherein in step (4), the method further comprises the steps of: applying an insulating coating and performing hot stretching leveling annealing.

In the method of the present invention, in some embodiments, before applying the insulating coating, an acid solution may be used to remove the unreacted components left on the surface of the steel plate after step (4), and then an insulating coating containing phosphate and colloidal silicon dioxide is coated and hot stretching leveling annealing is performed to finally obtain a high silicon grain-oriented electrical steel plate with excellent magnetic properties.

In addition, it should be noted that, in some embodiments, the cold spray treatment device for implementing step (2) of the method of the present invention includes: a gas tank, a gas control device, a particle conveyor, a gas heater, and a support roller with temperature control function, a nozzle device, a particle recovery device, a steel plate temperature detection device for measuring temperature of steel plate. The specific treating process of the cold spray device is described here. The working gas in the gas tank is transported to the gas heater through the gas control device; the working gas is heated by the gas heater and then transported to the nozzle device, and is accelerated in the nozzle device to form high speed jet. After the particle conveyor injects the high silicon alloy particles into the nozzle device, the high silicon alloy particles are accelerated to collision velocity by the high speed jet. When particles collide with the surface of the decarburization annealed steel plate to be sprayed at high speed, a high silicon alloy coating is formed on the surface of the steel plate to be sprayed. One or more nozzle devices can be arranged side-by-side around the support roller that are provided with temperature control function, so that the decarburization annealed steel plate to be sprayed is cold sprayed when running through the support roller, such that the treatment process of step (2) is achieved. In addition, the nozzle device can be fixed around the support roller or move back and forth along the width direction of the steel plate to be sprayed. The high silicon alloy particles left after colliding with the surface of the steel plate to be sprayed at high speed are collected by the particle recovery device.

Compared with the prior art, the method for manufacturing a high silicon grain-oriented electrical steel plate of the present invention has the following beneficial effects:

(1) The method for manufacturing a high silicon grain-oriented electrical steel plate of the present invention is based on conventional manufacturing lines and can mass-produce high silicon grain-oriented electrical steel plates by adding a set of cold spray treatment device, thereby solving the existing problem of high manufacturing cost.

(2) The method for manufacturing a high silicon grain-oriented electrical steel plate of the present invention enables high silicon alloy particles to be solid-deposited on the surface of the steel plate to be sprayed at a low temperature, which can significantly reduce or even completely eliminate adverse effects such as oxidation and phase transformation of high silicon alloy particles. Thereby, the stability of siliconizing during the annealing process of step (4) is ensured, and the problem of unstable quality of the high silicon steel plate in the existing manufacturing method is solved.

(3) The high silicon grain-oriented electrical steel plate manufactured by the method of the present invention has excellent magnetic properties, and the method has broad application prospects.

#### BRIEF DESCRIPTION OF DRAWINGS

FIG. 1 is a schematic view showing a structure of a cold spray treatment device for realizing the cold spray treatment process in the method for manufacturing the high silicon grain-oriented electrical steel plate of the present invention in some embodiments.

#### DETAILED DESCRIPTION OF INVENTION

The method for manufacturing the high silicon grain-oriented electrical steel plate of the present invention will be further explained and described in conjunction with the description of the drawings and specific embodiments. However, the explanation and the description do not improperly limit the technical solution of the present invention.

FIG. 1 is a schematic view showing a structure of a cold spray treatment device for realizing the cold spray treatment process in the method for manufacturing the high silicon grain-oriented electrical steel plate of the present invention in some embodiments. It can be seen that the cold spray treatment device for realizing the cold spray treatment process in the manufacturing method of the present invention includes: a gas tank 3, a gas control device 4, a particle conveyor 5, a gas heater 6, a support roller 7 with temperature control function, a nozzle device 8, a particle recovery device 9, and a steel plate temperature detection device 10 for measuring temperature of steel plate.

The specific working mode is described here. After a cold-rolled steel plate 1 undergoes decarburization annealing treatment in a decarburization annealing furnace 2, it enters the cold spray treatment device for treatment. The working gas in the gas tank 3 is transported to the gas heater 6 through the gas control device 4 (such as pipelines and valves); the working gas is heated by the gas heater 6 and then transported to the nozzle device 8, and is accelerated in the nozzle device 8 to form high speed jet. After the particle conveyor 5 injects the high silicon alloy particles into the nozzle device 8, the high silicon alloy particles are accelerated to collision velocity by the high speed jet. When particles collide with the surface of the decarburization annealed steel plate to be sprayed at high speed, a high

silicon alloy coating is formed on the surface of the steel plate to be sprayed. The nozzle device **8** is fixedly arranged around the support roller **7** that is provided with temperature control function, so that the decarburization annealed steel plate to be sprayed is cold sprayed when running through the support roller **7**. In addition, in some other embodiments, the nozzle device **8** can also move back and forth along the width direction of the steel plate to be sprayed. The high silicon alloy particles left after colliding with the surface of the steel plate to be sprayed at high speed are collected by the particle recovery device **9**. After the steel plate is cold sprayed, it enters a separation agent coating system **11** for subsequent processing.

Below, this technical solution will use specific example data to further describe the technical solution of this case and prove the beneficial effects of this case:

The steel billets in Example 1-24 and Comparative Example 1-15 use the same mass percentage of chemical elements.

Table 1 lists the mass percentages of the chemical elements of the steel billets of the high silicon grain-oriented electrical steel plates in Example 1-24 and Comparative Example 1-15.

TABLE 1

| (wt %, the balance is Fe and other unavoidable impurities) |       |      |       |       |        |
|------------------------------------------------------------|-------|------|-------|-------|--------|
| Si                                                         | C     | Mn   | S     | Als   | N      |
| 3.15                                                       | 0.046 | 0.11 | 0.005 | 0.030 | 0.0065 |

#### Examples 1-10 and Comparative Examples 1-5

The high silicon grain-oriented electrical steel plates of Examples 1-10 and Comparative Examples 1-5 were prepared by the following steps of:

(1) reheating the steel billet containing the mass percentage of each chemical element in Table 1 at 1050-1215° C., then hot rolling and annealing at 1050-1150° C. and pickling; thereafter rolling by a single stand mill;

(2) in an atmosphere of the mixture of humid nitrogen and hydrogen with a dew point of 40-65° C., performing a decarburization annealing with the cold-rolled steel plate at an annealing temperature of 820-850; controlling the total oxygen content on the surface of the decarburization annealed steel plate to be sprayed to be less than 700 ppm, and controlling element C content to be less than 50 ppm;

(3) ejecting the high silicon alloy particles and the heated working gas (nitrogen) of 400° C. onto the surface of the steel plate to be sprayed via a Laval nozzle with a conical inner surface so that making the high silicon alloy particles of complete solid state collide with the surface of the decarburization annealed steel plate to be sprayed at a speed of 500-900 m/s, thereinto, the high silicon alloy particles having a Si content of 10-50 wt %, the high silicon alloy particles having a particle size of 1-80 nm, the temperature of the high silicon alloy particles at the outlet of the nozzle being controlled as 300° C., and the outlet of the nozzle being set 25 mm away from the surface of the steel plate to be sprayed;

(4) coating a separation agent MgO and kiln drying;

(5) annealing: implementing a secondary recrystallization at an annealing temperature above 1100° C. in a N<sub>2</sub>+H<sub>2</sub> atmosphere, and then evenly heating the steel plate at a temperature above 1150° C. for at least 20 hours in a reducing atmosphere having a H<sub>2</sub> content over 90%;

(6) removing unreacted components left on the surface of the annealed steel plate via acid, then applying an insulating coating containing phosphate and colloidal silicon dioxide and performing hot stretching leveling annealing, so as to obtain the finished steel plate.

Table 2-1, Table 2-2, and Table 2-3 list the specific process parameters of the method for manufacturing the high silicon grain-oriented electrical steel plates of Examples 1-10 and Comparative Examples 1-5.

TABLE 2-1

| Serial number | Step(1)                                |                                                  |                                                           | Step (2)                                     |                                                                        |                                                                     |
|---------------|----------------------------------------|--------------------------------------------------|-----------------------------------------------------------|----------------------------------------------|------------------------------------------------------------------------|---------------------------------------------------------------------|
|               | Reheating temperature of billet (° C.) | Annealing temperature of hot rolled plate (° C.) | Dew point temperature of decarburization annealing (° C.) | Decarburization annealing temperature (° C.) | Total oxygen content on the surface of steel plate to be sprayed (ppm) | Element C content on the surface of steel plate to be sprayed (ppm) |
| Example 1     | 1083                                   | 1086                                             | 45                                                        | 840                                          | 503                                                                    | 15                                                                  |
| Example 2     | 1190                                   | 1141                                             | 60                                                        | 830                                          | 498                                                                    | 20                                                                  |
| Example 3     | 1125                                   | 1078                                             | 54                                                        | 830                                          | 398                                                                    | 39                                                                  |
| Example 4     | 1198                                   | 1144                                             | 60                                                        | 840                                          | 592                                                                    | 11                                                                  |
| Example 5     | 1116                                   | 1097                                             | 52                                                        | 820                                          | 481                                                                    | 25                                                                  |
| Example 6     | 1095                                   | 1149                                             | 64                                                        | 845                                          | 420                                                                    | 28                                                                  |
| Example 7     | 1118                                   | 1055                                             | 45                                                        | 840                                          | 357                                                                    | 41                                                                  |
| Example 8     | 1080                                   | 1087                                             | 55                                                        | 840                                          | 596                                                                    | 22                                                                  |
| Example 9     | 1061                                   | 1140                                             | 65                                                        | 835                                          | 440                                                                    | 13                                                                  |
| Example 10    | 1146                                   | 1100                                             | 52                                                        | 835                                          | 624                                                                    | 18                                                                  |
| Comparative   | 1132                                   | 1094                                             | 35                                                        | 815                                          | 339                                                                    | 53                                                                  |
| Example 1     |                                        |                                                  |                                                           |                                              |                                                                        |                                                                     |
| Comparative   | 1193                                   | <u>1000</u>                                      | 41                                                        | <u>855</u>                                   | 666                                                                    | 29                                                                  |
| Example 2     |                                        |                                                  |                                                           |                                              |                                                                        |                                                                     |
| Comparative   | 1215                                   | 1126                                             | 54                                                        | 830                                          | 541                                                                    | 20                                                                  |
| Example 3     |                                        |                                                  |                                                           |                                              |                                                                        |                                                                     |
| Comparative   | <u>1250</u>                            | 1056                                             | 62                                                        | 825                                          | 634                                                                    | 41                                                                  |
| Example 4     |                                        |                                                  |                                                           |                                              |                                                                        |                                                                     |
| Comparative   | 1201                                   | <u>1180</u>                                      | 70                                                        | 830                                          | <u>820</u>                                                             | 12                                                                  |
| Example 5     |                                        |                                                  |                                                           |                                              |                                                                        |                                                                     |

TABLE 2-2

| Serial number | Step(3)                                           |                                                    |                                                          |                                                 |                                                |                               |               |                |                     |
|---------------|---------------------------------------------------|----------------------------------------------------|----------------------------------------------------------|-------------------------------------------------|------------------------------------------------|-------------------------------|---------------|----------------|---------------------|
|               | Si content in high silicon alloy particles (wt %) | Particle size of high silicon alloy particles (μm) | Collision velocity of high silicon alloy particles (m/s) | Thickness of high silicon alloy coating Tc (μm) | Thickness of steel plate to be sprayed Ts (μm) | Target silicon content (wt %) | Spray surface | Tc/Ts          | (x1 - x2)/(x3 - x1) |
| Example 1     | 11.3                                              | 72                                                 | 757                                                      | 142                                             | 220                                            | 5.0                           | both sides    | 0.645          | 0.294               |
| Example 2     | 18.6                                              | 46                                                 | 849                                                      | 65                                              | 285                                            | 5.0                           | both sides    | 0.228          | 0.136               |
| Example 3     | 26.5                                              | 13                                                 | 684                                                      | 52                                              | 260                                            | 6.5                           | upper surface | 0.200          | 0.168               |
| Example 4     | 26.5                                              | 38                                                 | 684                                                      | 48.3                                            | 260                                            | 6.5                           | upper surface | 0.186          | 0.168               |
| Example 5     | 37.9                                              | 25                                                 | 686                                                      | 40.1                                            | 260                                            | 6.5                           | upper surface | 0.154          | 0.107               |
| Example 6     | 37.9                                              | 25                                                 | 628                                                      | 25.9                                            | 220                                            | 6.5                           | upper surface | 0.118          | 0.107               |
| Example 7     | 37.9                                              | 25                                                 | 618                                                      | 29.2                                            | 220                                            | 6.5                           | upper surface | 0.133          | 0.107               |
| Example 8     | 45.6                                              | 25                                                 | 615                                                      | 28.0                                            | 220                                            | 6.5                           | lower surface | 0.127          | 0.086               |
| Example 9     | 45.6                                              | 18                                                 | 531                                                      | 22.7                                            | 220                                            | 6.5                           | upper surface | 0.103          | 0.086               |
| Example 10    | 49.5                                              | 1.5                                                | 609                                                      | 21.3                                            | 220                                            | 6.5                           | upper surface | 0.097          | 0.078               |
| Comparative   | <u>55.8</u>                                       | 25                                                 | 685                                                      | <u>unbondi</u>                                  | 260                                            | 6.5                           | both sides    | <u>unbondi</u> | 0.68                |
| Example 1     |                                                   |                                                    |                                                          | <u>ng</u>                                       |                                                |                               |               | <u>ng</u>      |                     |
| Comparative   | <u>9.5</u>                                        | 25                                                 | 781                                                      | 200                                             | 260                                            | 6.5                           | both sides    | 0.769          | 1.117               |
| Example 2     |                                                   |                                                    |                                                          |                                                 |                                                |                               |               |                |                     |
| Comparative   | 36.5                                              | <u>81</u>                                          | <u>484</u>                                               | <u>unbondi</u>                                  | 260                                            | 6.5                           | both sides    | <u>unbondi</u> | 112                 |
| Example 3     |                                                   |                                                    |                                                          | <u>ng</u>                                       |                                                |                               |               | <u>ng</u>      |                     |
| Comparative   | 38.9                                              | <u>0.8</u>                                         | 673                                                      | <u>unbondi</u>                                  | 260                                            | 6.5                           | both sides    | <u>unbondi</u> | 103                 |
| Example 4     |                                                   |                                                    |                                                          | <u>ng</u>                                       |                                                |                               |               | <u>ng</u>      |                     |
| Comparative   | 37.9                                              | 10                                                 | 785                                                      | 15.8                                            | 260                                            | 6.5                           | upper surface | <u>0.061</u>   | 0.107               |
| Example 5     |                                                   |                                                    |                                                          |                                                 |                                                |                               |               |                |                     |

Among them, x1 is a target silicon content of the high silicon grain-oriented electrical steel plate, and its unit parameter is wt %; x2 is an initial silicon content of the steel plate to be sprayed, and its unit parameter is wt %; x3 is a silicon content of the high silicon alloy particles, and its unit parameter is wt %.

TABLE 2-3

| Serial number | Step(5)                                                     |                            |                                            |                          |
|---------------|-------------------------------------------------------------|----------------------------|--------------------------------------------|--------------------------|
|               | Annealing temperature of secondary recrystallization (° C.) | H <sub>2</sub> content (%) | High temperature of uniform heating (° C.) | Uniform heating time (h) |
| Example 1     | 1100                                                        | 95                         | 1175                                       | 36                       |
| Example 2     | 1100                                                        | 95                         | 1175                                       | 36                       |
| Example 3     | 1100                                                        | 95                         | 1200                                       | 28                       |
| Example 4     | 1120                                                        | 95                         | 1200                                       | 28                       |
| Example 5     | 1120                                                        | 100                        | 1200                                       | 28                       |
| Example 6     | 1120                                                        | 100                        | 1200                                       | 28                       |
| Example 7     | 1120                                                        | 100                        | 1220                                       | 24                       |
| Example 8     | 1150                                                        | 100                        | 1220                                       | 24                       |
| Example 9     | 1150                                                        | 100                        | 1220                                       | 24                       |
| Example 10    | 1150                                                        | 100                        | 1220                                       | 24                       |
| Comparative   | 1120                                                        | 100                        | 1200                                       | 28                       |
| Example 1     |                                                             |                            |                                            |                          |
| Comparative   | 1120                                                        | <u>85</u>                  | <u>1130</u>                                | 28                       |
| Example 2     |                                                             |                            |                                            |                          |
| Comparative   | 1120                                                        | 100                        | 1200                                       | 28                       |
| Example 3     |                                                             |                            |                                            |                          |
| Comparative   | 1120                                                        | 100                        | 1200                                       | 28                       |
| Example 4     |                                                             |                            |                                            |                          |
| Comparative   | 1120                                                        | 100                        | 1200                                       | <u>18</u>                |
| Example 5     |                                                             |                            |                                            |                          |

The performances of the high silicon grain-oriented electrical steel plates of Examples 1-10 and Comparative Examples 1-5 were tested for iron loss P<sub>10/400</sub>, magnetic induction B<sub>8</sub> and magnetostriction λ<sub>10/400</sub>. The test results are listed in Table 3.

TABLE 3

| Serial number | P <sub>10/400</sub> (W/Kg) | B <sub>8</sub> (T) | λ <sub>10/400</sub> (×10 <sup>-6</sup> ) | Si content in finished steel plate (wt %) |
|---------------|----------------------------|--------------------|------------------------------------------|-------------------------------------------|
|               |                            |                    |                                          | 30                                        |
| Example 1     | 7.5                        | 1.65               | 0.4                                      | 4.5                                       |
| Example 2     | 7.0                        | 1.57               | 0.3                                      | 5.6                                       |
| Example 3     | 6.7                        | 1.65               | 0.2                                      | 6.3                                       |
| Example 4     | 6.6                        | 1.47               | 0.1                                      | 6.7                                       |
| Example 5     | 6.4                        | 1.47               | 0.1                                      | 6.8                                       |
| Example 6     | 7.3                        | 1.67               | 0.3                                      | 6.0                                       |
| Example 7     | 6.3                        | 1.37               | 0.1                                      | 6.4                                       |
| Example 8     | 7.0                        | 1.40               | 0.1                                      | 6.7                                       |
| Example 9     | 5.7                        | 1.49               | 0.1                                      | 6.5                                       |
| Example 10    | 5.9                        | 1.37               | 0.1                                      | 6.9                                       |
| Comparative   | —                          | —                  | —                                        | —                                         |
| Example 1     | 8.7                        | 1.91               | 0.7                                      | 3.5                                       |
| Comparative   | —                          | —                  | —                                        | —                                         |
| Example 2     | —                          | —                  | —                                        | —                                         |
| Comparative   | —                          | —                  | —                                        | —                                         |
| Example 3     | —                          | —                  | —                                        | —                                         |
| Comparative   | —                          | —                  | —                                        | —                                         |
| Example 4     | 8.9                        | 1.91               | 0.6                                      | 3.7                                       |
| Example 5     |                            |                    |                                          |                                           |

It can be seen from Table 3 that all Examples 1-10 can obtain high silicon grain-oriented electrical steel plates with a silicon content higher than 4 wt %. The test results show that, compared with the finished steel plates with conventional silicon content, high-silicon steel plates have relatively low B<sub>8</sub> due to the increase in silicon content, while high-silicon steel plates have excellent high-frequency magnetic properties with high-frequency iron loss P<sub>10/400</sub> between 5.7-7.5 W/kg and magnetostriction λ<sub>10/400</sub> less than 0.4×10<sup>-6</sup>. Comparative Examples 1-5 cannot obtain the required high silicon grain-oriented electrical steel plates.

In order to verify the quality and performance of the sprayed steel plate, this technical solution includes Examples 11-20 and Comparative Examples 6-12. In Examples 11-20 and Comparative Examples 6-12, the high silicon grain-oriented electrical steel plate were sprayed by the following steps of:

11

(1) reheating the steel billet containing the mass percentage of each chemical element of Table 1 at 1050~1215°C., then hot rolling and annealing at 1050~1150°C. and pickling; thereafter cold rolling by a single stand mill to obtain a cold-rolled steel plate with a size of 0.285 mm;

(2) in an atmosphere of the mixture of humid nitrogen and hydrogen with a dew point of 40–65° C., performing a decarburization annealing with the cold-rolled steel plate at an annealing temperature of 820–850; controlling the total oxygen content on the surface of the decarburization annealed steel plate to be sprayed to be less than 700 ppm, and controlling element C content to be less than 50 ppm, so as to obtain a decarburization annealed steel plate with a size of 0.285 mm;

(3) ejecting the high silicon alloy particles and the heated working gas (such as nitrogen) onto the surface of the steel

12

plate to be sprayed via a Laval nozzle with a conical inner surface so that making the high silicon alloy particles of complete solid state collide with the surface of the decarburization annealed steel plate to be sprayed at a speed of 5 500-900 m/s, thereinto, the high silicon alloy particles having a Si content of 37.9 wt %, the high silicon alloy particles having a particle size of 20  $\mu\text{m}$ , the temperature of the high silicon alloy particles at the outlet of the nozzle being controlled as 80-500° C., and the outlet of the nozzle 10 being set 10-60 mm away from the surface of the steel plate to be sprayed; the Si content in the final high silicon grain-oriented electrical steel plate being expected to be 6.5 wt %.

Table 4-1 and Table 4-2 list the specific process parameters of the spraying and pre-spraying steps of Examples 11-20 and Comparative Examples 6-12.

TABLE 4-1

| Serial number | Step(1)                               |                                                  | Step (2)                                                 |                                              | Total oxygen                                              | Element C                                                 |
|---------------|---------------------------------------|--------------------------------------------------|----------------------------------------------------------|----------------------------------------------|-----------------------------------------------------------|-----------------------------------------------------------|
|               | Reheating temperature of billet(° C.) | Annealing temperature of hot rolled plate (° C.) | Dew point temperature of decarburization annealing(° C.) | Decarburization annealing temperature (° C.) | content on the surface of steel plate to be sprayed (ppm) | content on the surface of steel plate to be sprayed (ppm) |
| Example 11    | 1208                                  | 1114                                             | 47                                                       | 838                                          | 396                                                       | 23                                                        |
| Example 12    | 1185                                  | 1144                                             | 59                                                       | 823                                          | 514                                                       | 9                                                         |
| Example 13    | 1068                                  | 1059                                             | 59                                                       | 828                                          | 625                                                       | 29                                                        |
| Example 14    | 1099                                  | 1083                                             | 58                                                       | 848                                          | 558                                                       | 21                                                        |
| Example 15    | 1125                                  | 1120                                             | 56                                                       | 838                                          | 530                                                       | 27                                                        |
| Example 16    | 1200                                  | 1059                                             | 51                                                       | 833                                          | 634                                                       | 15                                                        |
| Example 17    | 1076                                  | 1137                                             | 57                                                       | 833                                          | 347                                                       | 20                                                        |
| Example 18    | 1087                                  | 1101                                             | 48                                                       | 833                                          | 529                                                       | 7                                                         |
| Example 19    | 1161                                  | 1129                                             | 53                                                       | 823                                          | 425                                                       | 48                                                        |
| Example 20    | 1085                                  | 1132                                             | 56                                                       | 838                                          | 586                                                       | 23                                                        |
| Comparative   | 1134                                  | 1138                                             | 50                                                       | 838                                          | 662                                                       | 17                                                        |
| Example 6     |                                       |                                                  |                                                          |                                              |                                                           |                                                           |
| Comparative   | 1060                                  | 1101                                             | 53                                                       | 843                                          | 668                                                       | 16                                                        |
| Example 7     |                                       |                                                  |                                                          |                                              |                                                           |                                                           |
| Comparative   | 1103                                  | 1085                                             | 46                                                       | 828                                          | 366                                                       | 24                                                        |
| Example 8     |                                       |                                                  |                                                          |                                              |                                                           |                                                           |
| Comparative   | 1091                                  | 1052                                             | 58                                                       | 828                                          | 394                                                       | 24                                                        |
| Example 9     |                                       |                                                  |                                                          |                                              |                                                           |                                                           |
| Comparative   | 1199                                  | 1065                                             | 59                                                       | 833                                          | 623                                                       | 14                                                        |
| Example 10    |                                       |                                                  |                                                          |                                              |                                                           |                                                           |
| Comparative   | 1196                                  | 1073                                             | 62                                                       | 843                                          | 623                                                       | 10                                                        |
| Example 11    |                                       |                                                  |                                                          |                                              |                                                           |                                                           |
| Comparative   | 1084                                  | 1076                                             | 45                                                       | 838                                          | 372                                                       | 24                                                        |
| Example 12    |                                       |                                                  |                                                          |                                              |                                                           |                                                           |

TABLE 4-2

TABLE 4-2-continued

| Serial number          | Working gas    | Collision velocity of high silicon alloy particles (m/s) | Temperature of high silicon alloy particles at the outlet of the nozzle (° C.) | Temperature of working gas (° C.) | Distance between the outlet of the nozzle and the surface of the steel plate to be sprayed (mm) | Spray surface | Step(3)                                        |                           |
|------------------------|----------------|----------------------------------------------------------|--------------------------------------------------------------------------------|-----------------------------------|-------------------------------------------------------------------------------------------------|---------------|------------------------------------------------|---------------------------|
|                        |                |                                                          |                                                                                |                                   |                                                                                                 |               | Thickness of high silicon alloy coating Tc(μm) | (x1 - x2)/Tc/Ts (x3 - x1) |
| Comparative Example 7  | N <sub>2</sub> | <u>915</u>                                               | 300                                                                            | 300                               | 25                                                                                              | both sides    | a little bonding unbonding                     | — 0.107                   |
| Comparative Example 8  | N <sub>2</sub> | 630                                                      | <u>62</u>                                                                      | <u>180</u>                        | 25                                                                                              | both sides    | —                                              | 0.107                     |
| Comparative Example 9  | N <sub>2</sub> | 630                                                      | 300                                                                            | <u>720</u>                        | 25                                                                                              | both sides    | 135.3                                          | 0.475 0.107               |
| Comparative Example 10 | N <sub>2</sub> | 630                                                      | <u>510</u>                                                                     | <u>720</u>                        | 25                                                                                              | both sides    | 158.9                                          | 0.558 0.107               |
| Comparative Example 11 | N <sub>2</sub> | 630                                                      | 300                                                                            | 550                               | <u>8</u>                                                                                        | both sides    | 125.6                                          | 0.441 0.107               |
| Comparative Example 12 | N <sub>2</sub> | 630                                                      | 300                                                                            | 550                               | <u>62</u>                                                                                       | upper surface | 25.8                                           | 0.091 0.107               |

Among them, x1 is a target silicon content of the high silicon grain-oriented electrical steel plate, and its unit parameter is wt %; x2 is an initial silicon content of the steel plate to be sprayed, and its unit parameter is wt %; x3 is a silicon content of the high silicon alloy particles, and its unit parameter is wt %.

The mass of the high silicon alloy coating of the high silicon grain-oriented electrical steel plates of Examples 11-20 and Comparative Examples 6-12 are listed in Table 5.

TABLE 5

| Serial number          | Mass of high silicon alloy coating                                      |
|------------------------|-------------------------------------------------------------------------|
| Example 11             | The coating thickness met the minimum requirements and was not oxidized |
| Example 12             | The coating thickness met the minimum requirements and was not oxidized |
| Example 13             | The coating thickness met the minimum requirements and was not oxidized |
| Example 14             | The coating thickness met the minimum requirements and was not oxidized |
| Example 15             | The coating thickness met the minimum requirements and was not oxidized |
| Example 16             | The coating thickness met the minimum requirements and was not oxidized |
| Example 17             | The coating thickness met the minimum requirements and was not oxidized |
| Example 18             | The coating thickness met the minimum requirements and was not oxidized |
| Example 19             | The coating thickness met the minimum requirements and was not oxidized |
| Example 20             | The coating thickness met the minimum requirements and was not oxidized |
| Comparative Example 6  | unbonding                                                               |
| Comparative Example 7  | a little bonding, coating oxidation                                     |
| Comparative Example 8  | unbonding                                                               |
| Comparative Example 9  | coating oxidation                                                       |
| Comparative Example 10 | coating oxidation                                                       |
| Comparative Example 11 | coating oxidation                                                       |
| Comparative Example 12 | coating was thin                                                        |

It can be seen from Table 5 that all Examples 11-20 can obtain required high silicon alloy coatings, while Comparative Examples 6-12 cannot obtain required high silicon alloy coatings.

The high silicon grain-oriented electrical steel plates of Examples 21-24 and Comparative Examples 13-15 were prepared by the following steps of:

(1) reheating the steel billet containing the mass percentage of each chemical element of Table 1 at 1050~1215° C., then hot rolling and annealing at 1050~1150° C. and pickling; thereafter cold rolling by a single stand mill to obtain a steel plate with the target thickness;

(2) in an atmosphere of the mixture of humid nitrogen and hydrogen with a dew point of 40~65° C., performing a decarburization annealing with the cold-rolled steel plate at an annealing temperature of 820~850; controlling the total oxygen content on the surface of the decarburization annealed steel plate to be sprayed to be less than 700 ppm, and controlling element C content to be less than 50 ppm;

(3) ejecting the high silicon alloy particles and the heated working gas (such as nitrogen) onto the surface of the steel plate to be sprayed via a Laval nozzle with a conical inner surface so that making the high silicon alloy particles of complete solid state collide with the surface of the decarburization annealed steel plate to be sprayed at a speed of 650 m/s, thereinto, the high silicon alloy particles having a Si content of 37.9 wt %, the high silicon alloy particles having a particle size of 20 μm, the temperature of the high silicon alloy particles at the outlet of the nozzle being controlled as 250° C., and the outlet of the nozzle being set 25 mm away from the surface of the steel plate to be sprayed;

(4) coating a separation agent MgO and kiln drying;

(5) annealing: implementing a secondary recrystallization at an annealing temperature above 1100° C. in a N<sub>2</sub>+H<sub>2</sub> atmosphere, and then evenly heating the steel plate at a temperature above 1150° C. for at least 20 hours in a reducing atmosphere having a H<sub>2</sub> content over 90%;

(6) removing unreacted components left on the surface of the annealed steel plate via acid, then applying an insulating coating containing phosphate and colloidal silicon dioxide and performing hot stretching leveling annealing, so as to obtain the finished steel plate.

Table 6-1, Table 6-2, and Table 6-3 list the specific process parameters of the method for manufacturing the high silicon grain-oriented electrical steel plates of Examples 21-24 and Comparative Examples 13-15.

TABLE 6-1

| Serial number | Step (1)                               |                                                  | Step (2)                                                  |                                              | Total oxygen content on the surface of steel plate to be sprayed (ppm) | Element C content on the surface of steel plate to be sprayed (ppm) |
|---------------|----------------------------------------|--------------------------------------------------|-----------------------------------------------------------|----------------------------------------------|------------------------------------------------------------------------|---------------------------------------------------------------------|
|               | Reheating temperature of billet (° C.) | Annealing temperature of hot rolled plate (° C.) | Dew point temperature of decarburization annealing (° C.) | Decarburization annealing temperature (° C.) |                                                                        |                                                                     |
| Example 21    | 1125                                   | 1060                                             | 45                                                        | 825                                          | 325                                                                    | 25                                                                  |
| Example 22    | 1090                                   | 1060                                             | 55                                                        | 825                                          | 423                                                                    | 27                                                                  |
| Example 23    | 1190                                   | 1070                                             | 60                                                        | 830                                          | 567                                                                    | 11                                                                  |
| Example 24    | 1100                                   | 1115                                             | 65                                                        | 835                                          | 665                                                                    | 36                                                                  |
| Comparative   | 1150                                   | 1100                                             | <u>68</u>                                                 | 840                                          | <u>750</u>                                                             | 19                                                                  |
| Example 13    |                                        |                                                  |                                                           |                                              |                                                                        |                                                                     |
| Comparative   | 1130                                   | 1150                                             | 65                                                        | 830                                          | <u>850</u>                                                             | 20                                                                  |
| Example 14    |                                        |                                                  |                                                           |                                              |                                                                        |                                                                     |
| Comparative   | 1180                                   | 1080                                             | 35                                                        | 830                                          | 403                                                                    | <u>72</u>                                                           |
| Example 15    |                                        |                                                  |                                                           |                                              |                                                                        |                                                                     |

TABLE 6-2

| Serial number | Working gas    | Step(3)                           |                                                |                               |               |                                                 |       |
|---------------|----------------|-----------------------------------|------------------------------------------------|-------------------------------|---------------|-------------------------------------------------|-------|
|               |                | Temperature of working gas (° C.) | Thickness of steel plate to be sprayed Ts (μm) | Target silicon content (wt %) | Spray surface | Thickness of high silicon alloy coating Tc (μm) | Tc/Ts |
| Example 21    | N <sub>2</sub> | 480                               | 220                                            | 6.5                           | upper surface | 47                                              | 0.213 |
| Example 22    | N <sub>2</sub> | 650                               | 220                                            | 6.5                           | upper surface | 28                                              | 0.130 |
| Example 23    | He             | 340                               | 260                                            | 6.5                           | both sides    | 78                                              | 0.298 |
| Example 24    | He             | 380                               | 260                                            | 6.5                           | both sides    | 75                                              | 0.289 |
| Comparative   | N <sub>2</sub> | 340                               | 220                                            | 6.5                           | upper surface | 45                                              | 0.204 |
| Example 13    |                |                                   |                                                |                               |               |                                                 |       |
| Comparative   | N <sub>2</sub> | 380                               | 220                                            | 6.5                           | upper surface | 53                                              | 0.242 |
| Example 14    |                |                                   |                                                |                               |               |                                                 |       |
| Comparative   | He             | 340                               | 260                                            | 6.5                           | both sides    | 61                                              | 0.236 |
| Example 15    |                |                                   |                                                |                               |               |                                                 |       |

Among them, x<sub>1</sub> is a target silicon content of the high silicon grain-oriented electrical steel plate, and its unit parameter is wt %; x<sub>2</sub> is an initial silicon content of the steel plate to be sprayed, and its unit parameter is wt %; x<sub>3</sub> is a silicon content of the high silicon alloy particles, and its unit parameter is wt %.

40 The content of element Si in the finished steel plates of the high silicon grain-oriented electrical steel plates of Examples 21-24 and Comparative Examples 13-15 are listed in Table 7.

TABLE 6-3

| Serial number | Step(5)                                                     |                            |                                            |                          |
|---------------|-------------------------------------------------------------|----------------------------|--------------------------------------------|--------------------------|
|               | Annealing temperature of secondary recrystallization (° C.) | H <sub>2</sub> content (%) | High temperature of uniform heating (° C.) | Uniform heating time (h) |
|               |                                                             |                            |                                            |                          |
| Example 21    | 1120                                                        | 92                         | 1175                                       | 32                       |
| Example 22    | 1140                                                        | 92                         | 1175                                       | 32                       |
| Example 23    | 1120                                                        | 100                        | 1200                                       | 28                       |
| Example 24    | 1140                                                        | 100                        | 1200                                       | 28                       |
| Comparative   | 1120                                                        | 92                         | 1175                                       | 32                       |
| Example 13    |                                                             |                            |                                            |                          |
| Comparative   | 1140                                                        | 92                         | 1175                                       | 32                       |
| Example 14    |                                                             |                            |                                            |                          |
| Comparative   | 1120                                                        | 100                        | 1200                                       | 28                       |
| Example 15    |                                                             |                            |                                            |                          |

45 TABLE 7

| Serial number | Content of element Si in finished steel plate (wt %) |
|---------------|------------------------------------------------------|
| Example 21    | 6.7                                                  |
| Example 22    | 6.1                                                  |
| Example 23    | 6.5                                                  |
| Example 24    | 6.7                                                  |
| Comparative   | 3.9                                                  |
| Example 13    |                                                      |
| Comparative   | 3.7                                                  |
| Example 14    |                                                      |
| Comparative   | 6.7                                                  |
| Example 15    |                                                      |

50 It can be seen from Table 7 that all Examples 21-24 can obtain high silicon grain-oriented electrical steel plates with required Si content, while the silicon content in the finished steel plates of comparative examples 13 and 14 are less than 4 wt %. The C content on the surface of the decarburization annealed steel plate to be sprayed of Comparative Example 55 60 65 66 67 68 69 70 71 72 73 74 75 76 77 78 79 80 81 82 83 84 85 86 87 88 89 810 811 812 813 814 815 816 817 818 819 820 821 822 823 824 825 826 827 828 829 830 831 832 833 834 835 836 837 838 839 840 841 842 843 844 845 846 847 848 849 850 851 852 853 854 855 856 857 858 859 8510 8511 8512 8513 8514 8515 8516 8517 8518 8519 8520 8521 8522 8523 8524 8525 8526 8527 8528 8529 8530 8531 8532 8533 8534 8535 8536 8537 8538 8539 8540 8541 8542 8543 8544 8545 8546 8547 8548 8549 8550 8551 8552 8553 8554 8555 8556 8557 8558 8559 8560 8561 8562 8563 8564 8565 8566 8567 8568 8569 8570 8571 8572 8573 8574 8575 8576 8577 8578 8579 8580 8581 8582 8583 8584 8585 8586 8587 8588 8589 8590 8591 8592 8593 8594 8595 8596 8597 8598 8599 85100 85101 85102 85103 85104 85105 85106 85107 85108 85109 85110 85111 85112 85113 85114 85115 85116 85117 85118 85119 85120 85121 85122 85123 85124 85125 85126 85127 85128 85129 85130 85131 85132 85133 85134 85135 85136 85137 85138 85139 85140 85141 85142 85143 85144 85145 85146 85147 85148 85149 85150 85151 85152 85153 85154 85155 85156 85157 85158 85159 85160 85161 85162 85163 85164 85165 85166 85167 85168 85169 85170 85171 85172 85173 85174 85175 85176 85177 85178 85179 85180 85181 85182 85183 85184 85185 85186 85187 85188 85189 85190 85191 85192 85193 85194 85195 85196 85197 85198 85199 85200 85201 85202 85203 85204 85205 85206 85207 85208 85209 85210 85211 85212 85213 85214 85215 85216 85217 85218 85219 85220 85221 85222 85223 85224 85225 85226 85227 85228 85229 85230 85231 85232 85233 85234 85235 85236 85237 85238 85239 85240 85241 85242 85243 85244 85245 85246 85247 85248 85249 85250 85251 85252 85253 85254 85255 85256 85257 85258 85259 85260 85261 85262 85263 85264 85265 85266 85267 85268 85269 85270 85271 85272 85273 85274 85275 85276 85277 85278 85279 85280 85281 85282 85283 85284 85285 85286 85287 85288 85289 85290 85291 85292 85293 85294 85295 85296 85297 85298 85299 85299 85300 85301 85302 85303 85304 85305 85306 85307 85308 85309 85310 85311 85312 85313 85314 85315 85316 85317 85318 85319 85320 85321 85322 85323 85324 85325 85326 85327 85328 85329 85330 85331 85332 85333 85334 85335 85336 85337 85338 85339 85340 85341 85342 85343 85344 85345 85346 85347 85348 85349 85350 85351 85352 85353 85354 85355 85356 85357 85358 85359 85360 85361 85362 85363 85364 85365 85366 85367 85368 85369 85370 85371 85372 85373 85374 85375 85376 85377 85378 85379 85380 85381 85382 85383 85384 85385 85386 85387 85388 85389 85390 85391 85392 85393 85394 85395 85396 85397 85398 85399 85399 85400 85401 85402 85403 85404 85405 85406 85407 85408 85409 85410 85411 85412 85413 85414 85415 85416 85417 85418 85419 85420 85421 85422 85423 85424 85425 85426 85427 85428 85429 85430 85431 85432 85433 85434 85435 85436 85437 85438 85439 85440 85441 85442 85443 85444 85445 85446 85447 85448 85449 85450 85451 85452 85453 85454 85455 85456 85457 85458 85459 85460 85461 85462 85463 85464 85465 85466 85467 85468 85469 85470 85471 85472 85473 85474 85475 85476 85477 85478 85479 85480 85481 85482 85483 85484 85485 85486 85487 85488 85489 85490 85491 85492 85493 85494 85495 85496 85497 85498 85499 85499 85500 85501 85502 85503 85504 85505 85506 85507 85508 85509 85510 85511 85512 85513 85514 85515 85516 85517 85518 85519 85520 85521 85522 85523 85524 85525 85526 85527 85528 85529 85530 85531 85532 85533 85534 85535 85536 85537 85538 85539 85540 85541 85542 85543 85544 85545 85546 85547 85548 85549 85550 85551 85552 85553 85554 85555 85556 85557 85558 85559 85560 85561 85562 85563 85564 85565 85566 85567 85568 85569 85570 85571 85572 85573 85574 85575 85576 85577 85578 85579 85580 85581 85582 85583 85584 85585 85586 85587 85588 85589 85590 85591 85592 85593 85594 85595 85596 85597 85598 85599 85599 85600 85601 85602 85603 85604 85605 85606 85607 85608 85609 85610 85611 85612 85613 85614 85615 85616 85617 85618 85619 85620 85621 85622 85623 85624 85625 85626 85627 85628 85629 85630 85631 85632 85633 85634 85635 85636 85637 85638 85639 85640 85641 85642 85643 85644 85645 85646 85647 85648 85649 85650 85651 85652 85653 85654 85655 85656 85657 85658 85659 85660 85661 85662 85663 85664 85665 85666 85667 85668 85669 85670 85671 85672 85673 85674 85675 85676 85677 85678 85679 85680 85681 85682 85683 85684 85685 85686 85687 85688 85689 85690 85691 85692 85693 85694 85695 85696 85697 85698 85699 85699 85700 85701 85702 85703 85704 85705 85706 85707 85708 85709 85710 85711 85712 85713 85714 85715 85716 85717 85718 85719 85720 85721 85722 85723 85724 85725 85726 85727 85728 85729 85730 85731 85732 85733 85734 85735 85736 85737 85738 85739 85740 85741 85742 85743 85744 85745 85746 85747 85748 85749 85750 85751 85752 85753 85754 85755 85756 85757 85758 85759 85760 85761 85762 85763 85764 85765 85766 85767 85768 85769 85770 85771 85772 85773 85774 85775 85776 85777 85778 85779 85780 85781 85782 85783 85784 85785 85786 85787 85788 85789 85790 85791 85792 85793 85794 85795 85796 85797 85798 85799 85799 85800 85801 85802 85803 85804 85805 85806 85807 85808 85809 85810 85811 85812 85813 85814 85815 85816 85817 85818 85819 85820 85821 85822 85823 85824 85825 85826 85827 85828 85829 85830 85831 85832 85833 85834 85835 85836 85837 85838 85839 85840 85841 85842 85843 85844 85845 85846 85847 85848 85849 85850 85851 85852 85853 85854 85855 85856 85857 85858 85859 85860 85861 85862 85863 85864 85865 85866 85867 85868 85869 85870 85871 85872 85873 85874 85875 85876 85877 85878 85879 85880 85881 85882 85883 85884 85885 85886 85887 85888 85889 85890 85891 85892 85893 85894 85895 85896 85897 85898 85899 85899 85900 85901 85902 85903 85904 85905 85906 85907 85908 85909 85910 85911 85912 85913 85914 85915 85916 85917 85918 85919 85920 85921 85922 85923 85924 85925 85926 85927 85928 85929 85930 85931 85932 85933 85934 85935 85936 85937 85938 85939 85940 85941 85942 85943 85944 85945 85946 85947 85948 85949 85950 85951 85952 85953 85954 85955 85956 85957 85958 85959 85960 85961 85962 85963 85964 85965 85966 85967 85968 85969 85970 85971 85972 85973 85974 85975 85976 85977 85978 85979 85980 85981 85982 85983 85984 85985 85986 85987 85988 85989 85990 85991 85992 85993 85994 85995 85996 85997 85998 85999 85999 85100 85101 85102 85103 85104 85105 85106 85107 85108 85109 85110 85111 85112 85113 85114 85115 85116 85117 85118 85119 85120 85121 85122 85123 85124 85125 85126 85127 85128 85129 85130 85131 85132 85133 85134 85135 85136 85137 85138 85139 85140 85141 85142 85143 85144 85145 85146 85147 85148 85149 85150 85151 85152 85153 85154 85155 85156 85157 85158 85159 85160 85161 85162 85163 85164 85165 85166 85167 85168 85169 85170 85171 85172 85173 85174 85175 85176 85177 85178 85179 85180 85181 85182 85183 85184 85185 85186 85187 85188 85189 85190 85191 85192 85193 85194 85195 85196 85197 85198 85199 85199 85200 85201 85202 85203 85204 85205 85206 85207 85208 85209 85210 85211 85212 85213 85214 85215 85216 85217 85218 85219 85220 85221 85222 85223 85224 85225 85226 85227 85228 85229 85230 85231 85232 85233 85234 85235 85236 85237 85238 85239 85240 85241 85242 85243 85244 85245 85246 85247 85248 85249 85250 85

It should be noted that the prior art part of the protection scope of the present invention is not limited to the embodiments given in this application document, and all prior arts that do not contradict the solution of the present invention, including but not limiting the previous patent documents, prior publications, prior public use, etc., can all be included in the protection scope of the present invention.

In addition, the combination of various technical features in this case is not limited to the combination described in the claims of this case or the combination described in the specific embodiments. All technical features described in this case can be freely combined or integrated in any way, unless conflicts arise among them.

It should also be noted that the embodiments listed above are only specific embodiments of the present invention. Obviously, the present invention is not limited to the above embodiments, and the subsequent similar changes or modifications that can be directly derived from or easily associated with the disclosure of the present invention by those skilled in the art, should fall within the protection scope of the present invention.

The invention claimed is:

1. A method for manufacturing a high silicon grain-oriented electrical steel plate, wherein the high silicon grain-oriented electrical steel plate has a silicon content of 25 greater than 4 wt %, the method comprising steps of:

- (1) performing a decarburization annealing to a cold-rolled steel plate, thereby forming a decarburization annealed steel plate;
- (2) spraying high silicon alloy particles of complete solid state collide on a surface of the decarburization annealed steel plate at a high speed of 500-900 m/s, so as to form a high silicon alloy coating on the surface of the decarburization annealed steel plate;
- (3) further coating a separation agent on the high silicon alloy coating from step (2) and drying; and
- (4) annealing.

2. The method for manufacturing a high silicon grain-oriented electrical steel plate according to claim 1, wherein in step (2), the high silicon alloy particles have a Si content of 10-50 wt %.

3. The method for manufacturing a high silicon grain-oriented electrical steel plate according to claim 1, wherein in step (2), the high silicon alloy particles have a particle size of 1-80  $\mu\text{m}$ .

4. The method for manufacturing a high silicon grain-oriented electrical steel plate according to claim 1, wherein in step (2), the high silicon alloy particles are driven by jet flow of working gas to collide.

5. The method for manufacturing a high silicon grain-oriented electrical steel plate according to claim 4, wherein the working gas is nitrogen, helium or mixture of nitrogen and helium.

6. The method for manufacturing a high silicon grain-oriented electrical steel plate according to claim 4, wherein the high silicon alloy particles and the working gas are ejected via a nozzle.

7. The method for manufacturing a high silicon grain-oriented electrical steel plate according to claim 6, wherein a temperature of the high silicon alloy particles at an outlet of the nozzle is controlled between 80-500° C.

8. The method for manufacturing a high silicon grain-oriented electrical steel plate according to claim 6, wherein the working gas is heated to 200-700° C. and then is sent to the nozzle.

9. The method for manufacturing a high silicon grain-oriented electrical steel plate according to claim 6, wherein the nozzle is a Laval nozzle.

10. The method for manufacturing a high silicon grain-oriented electrical steel plate according to claim 6, wherein the outlet of the nozzle is set 10-60 mm away from the 15 surface of the decarburization annealed steel plate.

11. The method for manufacturing a high silicon grain-oriented electrical steel plate according to claim 1, wherein the high silicon alloy coating is formed on one side or both sides of the surface of the decarburization annealed steel plate, and a thickness of the high silicon alloy coating satisfies the following formula:

$$T_c/T_s \approx (x_1 - x_2)/(x_3 - x_1)$$

wherein  $T_c$  is a thickness of the high silicon alloy coating, in  $\mu\text{m}$ , when the high silicon alloy coating is formed on both sides of the decarburization annealed steel plate, the thickness of the high silicon alloy coating is the sum of coating thickness of two sides of the decarburization annealed steel plate;  $T_s$  is a thickness of the decarburization annealed steel plate, in  $\mu\text{m}$ ;  $x_1$  is a target silicon content of the high silicon grain-oriented electrical steel plate, in wt %;  $x_2$  is an initial silicon content of the decarburization annealed steel plate, in wt %;  $x_3$  is a silicon content of the high silicon alloy particles, in wt %.

12. The method for manufacturing a high silicon grain-oriented electrical steel plate according to claim 1, wherein a total oxygen content on the surface of the decarburization annealed steel plate is controlled to less than 700 ppm, an element C content is controlled to less than 50 ppm, and a dew point of the decarburization annealing is controlled between 40-65° C.

13. The method for manufacturing a high silicon grain-oriented electrical steel plate according to claim 1, wherein in step (4), implementing a secondary recrystallization at an annealing temperature above 1100° C. and in a  $\text{N}_2 + \text{H}_2$  atmosphere, and then heating the coated decarburization annealed steel plate at temperature above 1150° C. for at least 20 hours and in a reducing atmosphere having a  $\text{H}_2$  content over 90%, so as to achieve a uniform diffusion of element Si.

14. The method for manufacturing a high silicon grain-oriented electrical steel plate according to claim 1, wherein after the step (4), the method further comprises the steps of: applying an insulating coating and performing hot stretching leveling annealing.

\* \* \* \* \*